

## UNITED STATES PATENT OFFICE

WILLIAM F. GEHRIG, OF BERKELEY HEIGHTS, NEW JERSEY, ASSIGNEE TO ESSEX SPECIALTY CO., INC., OF BERKELEY HEIGHTS, NEW JERSEY, A CORPORATION OF NEW JERSEY

## PYROTECHNICAL COMPOSITION

No Drawing. Application filed December 14, 1929. Serial No. 414,830.

This invention relates, generally, to pyrotechnical compositions; and the invention has reference, more particularly, to an improved non-detonating pyrotechnical or firework composition of the so called "snake" variety.

Heretofore, firework compositions of the "snake" variety have commonly contained picric acid as an essential ingredient. Owing to the strong tendency of picric acid to discolor objects in addition to its poisonous nature, firework compositions employing this acid are difficult to manufacture and pack for shipment due to the deleterious action of the acid on employees handling the firework composition. Such firework compositions are especially objectionable in use since children and others using the same get their hands and clothes badly discolored and also because of the poisonous nature of the picric acid constituent. Other firework compositions of the above character which have been used employ poisonous mercury as an essential ingredient, thereby rendering the firework dangerous in use.

The principal object of the present invention is to provide a novel firework composition of the "snake" variety that eliminates the use of picric acid and mercury and employs only such harmless constituents which when combined, in the proper proportions hereinafter stated, produce a harmless firework which will not discolor the hands or clothes and which does not have the poisonous characteristics common to fireworks of the "snake" variety.

Another object of the present invention lies in the provision of a firework composition of the above character that is non-hygroscopic, which remains stable indefinitely, is readily ignited in use and which produces an excellent snake formation; and to this end use is made of nitrated coal tar naphthol pitch to provide the enveloping body for the firework, tetryl is employed for producing the necessary gas

for expanding the enveloping body, and nitro-cellulose is used for aiding and distributing the combustion throughout the mass of the firework. Tetryl, as the active gas producing agent, is especially important in forming the firework composition since this substance produces heat and gas at the relatively slow desired rate for accomplishing the purposes of the firework. Also, suitable lubricators in the form of either graphite or stearic acid or both are included in the composition to facilitate its compression in and removal from molds, whereby firework buttons or tablets are produced for use.

In making up the novel firework composition of this invention, linseed oil is added to a coal tar pitch known in the trade as naphthol pitch and nitric acid is then added to this mixture causing a vigorous reaction. Fish oil or other suitable oil may be used in lieu of linseed oil in carrying out this reaction but the use of such an oil is essential to carry on the nitration of the naphthol pitch. The resulting porous pitch mass is allowed to dry and provides a nitrated naphthol pitch which is then granulated or ground to small particles whereupon the remaining ingredients consisting of tetryl, a lubricant such as stearic acid or graphite or both, and finally nitro-cellulose are added and the resulting composition compressed into small buttons or pellets for use.

As an example of the composition of this invention, the ingredients are mixed together in the following proportions by weight:

|                                | Parts |
|--------------------------------|-------|
| Naphthol pitch (beta) -----    | 300   |
| Linseed oil (raw) -----        | 60    |
| Nitric acid (commercial) ----- | 250   |
| Tetryl -----                   | 100   |
| Stearic acid -----             | 1/2   |
| Graphite -----                 | 1/2   |
| Nitro-cellulose -----          | 20    |
|                                | 90    |

The preferred manner of preparing the composition is as follows:

Three hundred ounces of coal tar naphthol pitch preferably of the beta variety in fine granular form is placed in a crock or other suitable container and sixty ounces of raw linseed oil is then poured over this granular naphthol pitch. The linseed oil films over the naphthol pitch granules. Two hundred and fifty ounces of nitric acid, preferably of ordinary commercial strength, is then added to the mixture in the crock and a vigorous reaction thereupon takes place with the liberation of heat. During this reaction, which lasts about ten minutes, the contents of the crock are stirred continuously, thereby liberating the fumes formed during the reaction, such fumes, so far as is now known, carrying off the oil. After the reaction has ceased, the resulting mass of material provides the nitrated naphthol pitch, which is an essential ingredient of the final composition. This nitrated naphthol pitch is allowed to dry at ordinary temperatures, which usually takes from one to two days; after which the dried mass of naphthol pitch is ground to small particles or granules. To this resultant granular mass of nitrated naphthol pitch is added one-hundred ounces of tetryl, which is also used in the form of small granules. One-half ounce of powdered stearic acid and one-half ounce of powdered graphite, being the preferred form of lubricator agent, is thereupon added. Finally, twenty ounces of nitro-cellulose in its common dry fluffy form is added and the several substances are thoroughly mixed together as by stirring. The resulting composition is then compressed in molds to combine the several ingredients into a unitary mass and to produce small buttons or pellets ready for use. The stearic acid and the graphite assist greatly in the molding process by serving as lubricants for the several constituents of the firework composition as well as by lubricating the relatively movable parts of the mold, thereby preventing the breaking of the buttons or pellets while being removed from the mold.

The firework composition thus produced has the form of a relatively hard dense mass which does not tend to crumble and is non-hygroscopic, is stable and keeps well under variations of climatic or weather conditions, is not subject to spontaneous combustion and in use is readily ignited to produce an exceptionally profuse and lengthy "snake" of uniform diameter and density and of highly attractive and amusing qualities.

The nitrated naphthol pitch provides the expandable body of the firework, tetryl, as the active agent, provides the expanding gases together with a certain amount of heat, nitro-cellulose distributes and enhances the burning, and the stearic acid and graphite serve as lubricants in forming the firework buttons

and the former also by burning serving as an aid in distributing the combustion.

While in the above illustrative table there is given the relative proportions of the several ingredients of the composition, it will be understood that variation of the stated proportions may be made within reasonable limits. For example, by increasing the relative proportions of nitrated naphthol pitch while keeping the quantities of the other constituents the same, the length of the resulting "snake" will be increased while the rate of combustion of the composition and hence the rate at which the "snake" is formed will be slower than before; while, on the other hand, by decreasing the relative proportions of the nitrated naphthol pitch while keeping the other constituents the same, the rate of combustion of the composition will be increased though a shorter "snake" will be produced.

Also by varying the tetryl ingredient the rapidity with which the "snake" is formed will be correspondingly varied. Varying of the nitro-cellulose ingredient varies the uniformity and rapidity of the burning, i. e. by increasing the relative proportion of this ingredient the burning is more rapid and uniform while lessening this ingredient has the reverse effect.

Having thus described the invention, what is claimed is:

1. A firework composition of the class described comprising, nitrated naphthol pitch together with tetryl, the nitrated naphthol pitch providing in use an enveloping expandable body and the tetryl providing gases for expanding said body.

2. A firework composition of the class described comprising, an expandable body consisting of nitrated naphthol pitch together with tetryl as an active agent and nitro-cellulose as a heat dispersive agent.

3. A firework composition of the class described comprising, an expandable body consisting of nitrated naphthol pitch, tetryl as an active gas producing agent, and a lubricant.

4. A firework composition of the class described comprising, an expandable body consisting of nitrated naphthol pitch, tetryl as an active gas producing agent, nitro-cellulose and a lubricant.

5. A firework composition of the class described comprising, an expandable body consisting of nitrated naphthol pitch, tetryl as an active gas producing agent, nitro-cellulose as a heat dispersive agent and graphite.

6. A firework composition of the class described comprising, an expandable body consisting of nitrated naphthol pitch, tetryl as an active gas producing agent, nitro-cellulose as a heat dispersive agent and stearic acid.

7. A firework composition of the class described comprising, an expandable body consisting of nitrated naphthol pitch, tetryl as an

active gas producing agent, nitro-cellulose, stearic acid and graphite.

8. A composition for production of a fire-work of the class described comprising the 5 herein named ingredients in the approximate proportions by weight as follows:—

|                                  | Parts         |
|----------------------------------|---------------|
| Naphthol pitch (beta)-----       | 300           |
| Linseed oil (raw)-----           | 60            |
| 10 Nitric acid (commercial)----- | 250           |
| Tetryl-----                      | 100           |
| Stearic acid-----                | $\frac{1}{2}$ |
| Graphite-----                    | $\frac{1}{2}$ |
| 15 Nitro-cellulose-----          | 20            |

In testimony, that I claim the invention set forth above I have hereunto set my hand this 9th day of December, 1929.

WILLIAM F. GEHRIG.

20

25

30

35

40

45

50

55

60

65